

March 17, 1964

R. WOODELL

3,124,926

BULKY YARN

Filed Oct. 24, 1962

3 Sheets-Sheet 1

*Fig. 1*



INVENTOR  
RUDOLPH WOODELL

BY *William Petty*

ATTORNEY

March 17, 1964

R. WOODELL

3,124,926

BULKY YARN

Filed Oct. 24, 1962

3 Sheets-Sheet 2

*Fig. 2*



*Fig. 3*



INVENTOR

RUDOLPH WOODELL

BY

*William Petty*

ATTORNEY

March 17, 1964

R. WOODELL

3,124,926

BULKY YARN

Filed Oct. 24, 1962

3 Sheets-Sheet 3

FIG. 4



FIG. 5



INVENTOR

RUDOLPH WOODELL

BY

*Harry E. Bradlock*

ATTORNEY

## 1

3,124,926  
BULKY YARN

Rudolph Woodell, Richmond, Va., assignor to E. I. du Pont de Nemours and Company, Wilmington, Del., a corporation of Delaware

Filed Oct. 24, 1962, Ser. No. 233,205

5 Claims. (Cl. 57—140)

This invention relates to a novel and useful bulky yarn composed of continuous filaments and a process and apparatus for its production. This is a continuation-in-part of my copending application Serial No. 757,230, filed August 26, 1958.

Almost all synthetic fibers are produced most easily as continuous filaments. Continuous filament yarns are much stronger than staple fiber yarns because of the absence of loose ends but, because of their extreme uniformity and lack of discontinuities, conventional continuous filament yarns are much more dense than their staple counterparts. The filaments lie close together in the yarn, and adjacent strands of continuous filament yarn in fabrics are closely and evenly spaced. It would be desirable to provide a continuous filament yarn which retains its strength characteristics and which has the lightness and covering effectiveness, as well as interesting decorative surface effects, commonly achieved with yarns spun from staple fibers.

U.S. Patent 2,783,609, issued to A. L. Breen on March 5, 1957, discloses one process for converting continuous filament yarn into bulky yarn which, when woven into fabrics, gives effects similar to those obtained with staple yarns. In this process the continuous filament yarn is passed through a turbulent stream of air or other gas where the filaments are looped and entangled to give the desired bulk. While this process produces very desirable bulky continuous filament yarns, it obviously requires that the yarn be prepared in the conventional manner, and then be subsequently subjected to a second operation in order to obtain the final product. In addition, fabrics made from this yarn have a uniform surface appearance and are, therefore, not as susceptible to the formation of non-uniform, decorative surface effects.

Decorative surface effects in fabrics have frequently been achieved by the use of slub yarns, i.e. yarns having bulky protrusions at intervals along their length. The slub yarns of the prior art, however, tend to be uniform with regard to the size and spacing of the slubs. Furthermore, known processes which provide slub yarns do not readily yield slubs of considerable length, i.e. four to five inches.

It is an object of this invention to provide a novel and useful bulky, continuous filament yarn. Another object is to provide a novel bulky yarn which may be used to produce fabrics having unique, decorative surface effects. Another object is to provide a process and apparatus for producing the yarn. Other objects will become apparent from the specification and claims.

According to this invention, there is provided a yarn composed of continuous filaments in which the filaments are looped and entangled at intervals throughout the filament length to form bulky sections in the yarn, the bulky sections varying in a random fashion with respect to length, bulkiness and spacing along the yarn, the minimum variation in length being at least five-fold and the minimum variation in bulkiness being at least two-fold, i.e. the longest bulky section is at least five times the length of the least bulky section and the average diameter of the most bulky section is at least twice the average diameter of the least bulky section. The variations in bulkiness and in the length of the bulky sections which result from this treatment, as well as the occurrence of

## 2

short non-bulky sections of varying length, enhance the decorative effects obtained when the yarn is woven into fabric.

This novel bulky yarn is produced by feeding a plurality of continuous filaments into a rapidly moving stream of liquid, introducing the filaments and liquid into a chamber, imparting a turbulent swirling motion to the liquid containing the filaments to carry the filaments in a generally circular path within the chamber and to entangle the filaments, and drawing the filaments away under low tension.

The feed yarn is any continuous multifilament yarn from a suitable source, such as a conventional package, and is preferably supplied at substantially zero twist. The feed filaments can be introduced directly from a wet-spinning operation, in which case an effective process comprises extruding a filament-forming solution through a spinneret assembly into a coagulating solution to form a plurality of filaments, introducing (preferably concurrently) the newly-formed filaments into a rapidly moving stream of liquid, preferably a coagulating liquid, whereby the filaments are carried into a chamber, imparting a turbulent swirling motion to the liquid to carry the filaments in a generally circular path, preferably about three-quarters of the way around the chamber, and to entangle the filaments, and thereafter drawing the filaments away under low tension.

According to one embodiment of the invention, a novel blended bulky yarn is provided by introducing other filaments, preferably synthetic filaments, into the rapidly moving stream of coagulating liquid along with the newly-formed filaments.

Apparatus utilizing wet-spinning for producing the yarns comprises a spinneret, means for supplying a filament-forming solution to the spinneret, a conduit through which the filaments pass after extrusion from the spinneret, means for forcing liquid, preferably a coagulating liquid through the conduit along with the filaments, a chamber situated at the end of the conduit to receive the filaments and coagulating liquid, the chamber having an outlet for the liquid and filaments and means for imparting to the liquid in the chamber a turbulent swirling motion. Apparatus suitable for processing prespun yarn differs only in that the spinneret and means for supplying filament-forming solution are replaced by conventional means for feeding yarn to the conduit from a package or other convenient source.

FIG. 1 is a schematic isometric drawing of a typical form of apparatus suitable for performing the process of this invention.

FIG. 2 is a transverse cross-section of the swirl pool shown schematically in FIG. 1.

FIGURE 3 is a cross-section along the line 3—3 of FIGURE 2.

FIGURE 4 is a magnified partial longitudinal side view of a yarn embodying the present invention.

FIGURE 5 is a less magnified view of the yarn of FIGURE 4.

In the apparatus shown in FIGURE 1, a filament-forming solution is extruded through spinneret 1 into a coagulating and regenerating bath 2 which partially fills spin box 3. The freshly formed filaments 4 are carried downwardly through spinning tube 5 by a rapidly moving stream of the coagulating bath which is forced through the tube 5 by the pressure head of the coagulating and regenerating bath which surrounds spinneret 1 and entrance of spinning tube 5. The bath carrying the filaments is discharged into swirl pool 6 and is given a swirling motion by a second stream of bath from container 7 fed from spin box 3 and through conduit 13. This bath is jetted through conduit 14 and orifice 8 (as

shown in FIGURE 3) at an angle with respect to the exit of spinning tube of about 90°. The velocity of the bath through the orifice 8 is adjusted to impart a swirling motion of sufficient intensity to deflect the filaments and carry them in a generally circular path about three-quarters of the way around the chamber (as shown in FIGURE 3) before being discharged through the opening 9 in the bottom of the chamber. The yarn is discharged from the chamber 6 into the discharge tube 11 from which it passes for a distance through the bath 20 in container 12 over a converging guide 16 and through various other guides 17 and 18, and finally to a conventionally centrifugal spinning bucket (not shown) where the yarn is wound into a cake in the conventional manner.

A transverse enlarged cross-section of the container or swirl pool 6 of FIGURE 1 is shown in FIGURE 2.

FIGURE 3 shows the normal path of filament movement in swirl pool 6. The swirl pool 6 has an inner opening, shown in FIGURE 3 as bowl-shaped chamber 6. The exit of the spinning tube 5 leads into chamber 6 off-center of the axis of revolution of the chamber and orifice 8 of the bath jet is located in line with the exit of spinning tube 5, at an angle of about 90° with its axis. Opening 9 in the bottom of the chamber leads into discharge tube 11, which is curved at a 90° angle outside the container into the bath 20. Pin 10 holds the discharge tube securely in place.

#### EXAMPLE I

Viscose containing 6.25% recoverable cellulose and 5.75% alkali, calculated as sodium hydroxide, is prepared in the conventional manner from cotton linters pulp using 30% carbon disulfide based on the air dry weight of the pulp. The viscose is filtered, deaerated, ripened to a salt index of 4.3 and a viscosity of about 55 poises and extruded through a spinneret having 120 holes of 0.0025 inch diameter into a coagulating and regenerating bath containing 9.5% sulfuric acid, 19.25% sodium sulfate, 3.5% zinc sulfate, 2.0% glucose and maintained at a temperature of 55° C.

The freshly formed filaments are passed through a spinning tube of 7 mm. diameter for a distance of 9 inches by a rapidly moving stream of coagulating bath which is forced through the tube by maintaining a bath head of about 9 inches in a container which surrounds the spinneret and tube entrance. The bath carrying the filaments is discharged into a bowl shaped chamber 3 inches in diameter and 2.5 in. deep. A second stream of bath is jetted through an orifice of 0.1875 inch diameter under a pressure head of about 115 inches of bath. The second bath stream is jetted into the first bath stream carrying the uncoagulated filaments at an angle of about 90° with respect to the exit of the spinning tube.

The velocity of the bath through the orifice is adjusted to impart a swirling motion of sufficient intensity to deflect the filaments and carry them in a generally circular path about three-quarters of the way around the chamber before being discharged through the opening in the bottom of the chamber. The yarn is then carried for a distance of about 7 inches through a tube of 12 mm. diameter. The yarn is then passed for six inches through a coagulating and regenerating bath, of the composition given above, over a Y-guide and then for a further distance of 33 inches through the bath where it is confined by means of two roller guides. The yarn is then passed under a hook guide, up to and around a feed wheel having a peripheral speed of 90 yards per minute and then downwardly into a centrifugal spinning bucket where the yarn, which has an average denier of 300, is wound into a cake in the conventional manner.

The yarn is purified, dried and wound into cones in the conventional manner. The yarn contains bulky sections varying in length from about 1/2 inch to about 6 inches. The average diameter (bulkiness) of the most

bulky sections is at least 3 times that of the least bulky sections. The longer bulky sections vary appreciably in bulkiness along their length. The non-bulky sections vary in length from about 1/2 inch to about 3 to 4 inches to give a random spacing of the bulky portions of the yarn. When the yarn is woven into a plain weave fabric the fabric has the desirable texture of a fabric woven from spun yarn and in addition displays a linen-like effect due to the random variation in bulkiness of the yarn. Very desirable linen-like fabric is obtained when the above yarn is used as a filling in a plain weave fabric with a cotton warp.

#### EXAMPLE II

Viscose containing 6.25% recoverable cellulose and 5.75% alkali, calculated as sodium hydroxide, is prepared in the conventional manner from cotton linters pulp using 30% carbon disulfide based on the air dry weight of the pulp. The viscose is filtered, deaerated, ripened to a salt index of 4.0 and a viscosity of about 55 poises and extruded through a spinneret having 120 holes of 0.0035 inch diameter into a coagulating and regenerating bath containing 9.5% sulfuric acid, 19.25% sodium sulfate, 3.5% zinc sulfate and 2.0% glucose, the temperature of the bath being 55° C.

The freshly formed filaments are carried downwardly through a spinning tube of 7 mm. diameter and 14 inches length by a rapidly moving stream of coagulating bath which is forced through the tube by maintaining the bath level about 1 to 2 inches above the tube entrance in the container which surrounds the spinneret and tube entrance. The bath carrying the filaments is discharged into a bowl-shaped circular chamber 2 1/2 inches in diameter and having an average depth of 1 15/32 inches. A second stream of bath is jetted through an orifice of 0.1875 inch diameter into the first bath stream carrying the uncoagulated filaments, the angle of the bath jet with respect to the spinning tube exit being about 90°.

The velocity of the bath through the orifice is adjusted to impart a swirling motion of sufficient intensity to deflect the filaments and carry them in a generally circular path about three-quarters of the way around the chamber before being discharged through the opening in the bottom of the chamber. The yarn is discharged from the bowl into a tube of 13 millimeters inside diameter and an over-all length of 7 inches. After leaving the tube which is submerged in coagulating bath, the yarn is passed for a distance of 6 inches through the bath, over a Y-guide, and then for a further distance of 33 inches through the bath where it is confined by means of a roller guide. The yarn is then passed under a hook guide, up to and around a feed wheel having a peripheral speed of 90 yards per minute and then downwardly into a centrifugal spinning bucket where the yarn, which has an average denier of 300, is wound into a cake in the conventional manner.

The yarn is purified, dried and wound into cones in the conventional manner. The yarn contains bulky sections varying in length from about 1/2 inch to 6 inches. The average diameter of the most bulky sections is judged to be at least 3 times that of the least bulky sections. The non-bulky sections vary in length from about 1/2 inch to about 3 to 4 inches to give a random spacing of the bulky sections. The longer bulky sections vary appreciably in bulkiness along their length. When the yarn is woven into a plain weave fabric, the fabric has the desirable texture of a fabric woven from spun yarn and in addition, displays a linen-like effect due to the random variation in bulkiness of the yarn. Very desirable linen-like fabric is obtained when the above yarn is used as a filling in a plain weave fabric with a cotton warp.

#### EXAMPLE III

Example I is repeated except that a zero twist polyethylene terephthalate yarn is fed into the top of the

spinning tube, combined with the rayon filaments, and carried through the process. By this means, the rayon and polyethylene terephthalate filaments are intermingled to produce a bulky blended yarn. The yarn is similar in general appearance to the yarn of Example II. Various deniers of rayon are combined with the various deniers of polyethylene terephthalate yarn to produce the combinations shown in Table I below:

Table I

| Rayon (Total denier) | Polyethylene terephthalate (Total denier) | Percent Polyethylene terephthalate |
|----------------------|-------------------------------------------|------------------------------------|
| 230                  | 70                                        | 23                                 |
| 70                   | 30                                        | 30                                 |
| 70                   | 70                                        | 50                                 |
| 30                   | 70                                        | 70                                 |

When the 300 denier yarn containing 23% polyethylene terephthalate yarn is woven into fabric, an attractive spun-like fabric of high bulk is obtained. The major portion of the rayon and polyethylene terephthalate filaments appear to be intimately mixed, however, the slubs in the fabrics have been found to be either polyethylene terephthalate rayon, or a mixture of polyethylene terephthalate and rayon so that crossdyeing gives unusual splash effects. The other yarns listed in Table I also produce attractive fabrics.

## EXAMPLE IV

Apparatus similar to that used in Example II is set up except that a spinneret is not used and water is used as the liquid bath instead of a coagulating bath. A 100 denier, 68 filament, 0 twist yarn, of polyethylene terephthalate including 2 mol percent of the sodium salt of poly(sulfisophthalate), the filaments having a trilobal cross-section, is fed to the spinning tube of the spinning box. The yarn, as it comes from the supply package, is led through a tension gate and is passed through a spinning tube of 0.25 inch diameter and 14 inches in length. The yarn is fed to the bowl-shaped chamber by the rapidly moving stream of water, which is forced by gravity through the tube by maintaining the bath level in the spin box about 1 to 2 inches above the tube entrance. The tension gate is adjusted to supply a low level of tension to the yarn so as to minimize tension variations resulting from take-off from the supply package. The water passing down the spinning tube carries the filaments to a bowl-shaped circular chamber 2.875 inches in diameter and having an average depth of about 1.5 inches. A second stream of water is carried from container 7, which is located about 5 inches above the height of the water in container 12, and is jetted through orifice 8 having a diameter of 0.1875 inch into the first bath stream carrying the unconverted filaments, the angle of the bath jet with respect to the spinning tube exit being about 90 degrees.

The velocity of the water through orifice 8 is adjusted to impart a swirling motion to the water in the bowl-shaped chamber but not of sufficient velocity to cause the water to overflow from the chamber. The swirling action is of sufficient intensity to deflect the filaments and carry them in a general circular path about  $\frac{3}{4}$  of the way around the chamber before they are discharged through the 0.5 inch opening in the bottom of the chamber. The yarn then passes from the bowl into tube 11 of 0.375 inch inside diameter and having a length of about 6 inches. After leaving the tube which is submerged in the water in container 12, the yarn passes for a distance of about 20 inches through the water and is led through a pigtail guide before exiting from the bath. Since the windup speed is less than the speed at which the slubbed yarn is discharged from tube 11, additional entanglement of the yarn occurs between the exit of tube 11 and the pigtail guide. After exiting from the bath, the yarn passes

around a convenient snubbing device, such as a spool guide, in order to apply a slight tension between the yarn and the windup. After passing over the spool guide, the yarn is led to the windup where it is wound into a package in a conventional manner at a windup speed of 27 yards per minute.

The yarn, which has an average denier of 251.8, contains bulky sections varying in length from 0.25 to 28 inches with an average length of 3.8 inches. The bulky sections, of which there are 200 to 230 per 100 yards, have a maximum denier of 800. The interval between the bulky sections varies from 1 to 72 inches with an average of 14 inches.

When the above experiment is repeated using an aqueous spin-finish emulsion, essentially equivalent results are obtained.

## EXAMPLE V

Example IV is repeated except that the yarn is wound up at a speed of 48 yards per minute. At this windup speed the bulky sections are formed within the bowl-shaped chamber and no additional entanglement occurs in bath 21.

The yarn, which has an average denier of 113.1, contains bulky sections varying in length from about 0.5 to 12 inches with an average length of about 3 inches. The bulky sections have a maximum denier of 450 and there are 87 to 93 bulky sections per 100 yards. The interval between the bulky sections varies in length from 6 to 144 inches with an average of 37 inches.

## EXAMPLE VI

Example V is repeated except that a 40-denier, 27 filament yarn is added as a support yarn. The filaments of the support yarn have a trilobal cross-section and are melt spun from a polyethylene terephthalate copolymer having 2 mol percent of the sodium salt of poly(sulfisophthalate).

The support yarn is removed from the supply package and passes over a guide and is then fed to the vortex of the whirlpool and follows the same path to the windup as does the yarn having the bulky portions. The component of the combined yarn that contains the bulky portions is the same as that of Example V. The yarn containing the bulky portions and the support yarn are well combined. The average denier of the combined yarn is 152.8.

Any filament-forming solution is suitable for treatment in accordance with this invention. Viscose solutions which are commonly used in the spinning of textile rayons are particularly satisfactory. In addition, cuprammonium solutions of cellulose and other filament-forming solutions such as cellulose acetate and polyacrylonitrile solutions, conventionally used in wet spinning processes, can be satisfactorily employed in the process of this invention. Likewise, any of the coagulating liquids commonly used in wet spinning process may be satisfactorily employed. In the viscose process, baths containing 4-12% sulfuric acid, sodium sulfate and other metal sulfates such as zinc sulfate are commonly used and are suitable.

Any other continuous filament feed from a different source may be intermingled with the wet-spun filaments to provide the novel blended bulky yarn, or can entirely replace wet-spun filaments to produce bulky yarn products of this invention. For example, yarns comprising polyesters, such as polyethylene terephthalate, polyamides such as the conventional nylons, dry-spun acrylonitrile polymers, polyurethanes, poly (vinyl chloride) polymers and copolymers thereof are suitable.

The velocity of the bath in the conduit leading away from the spinneret or other source of feed yarn may be adjusted to any speed depending on the processing speed desired. In commercial practice, the velocity is preferably fairly high, i.e., 40 yds./min. or higher, since the

filaments are carried solely by the bath, the higher the velocity, the higher the processing speed, of course. Also, in the event that the swirling motion in the chamber at the end of the tube is imparted by the use of a baffle which directs the bath flow towards the wall of a circular chamber, then the velocity should be sufficiently high to provide an adequate swirling motion within the chamber. Preferably, the swirling motion should be adjusted to carry the filaments about three-fourths of the way around the chamber, that is, they traverse about three-quarters of a circle before being discharged from the chamber into the exit tube.

The turbulent swirling motion in the chamber at the end of the conduit may be created in a number of ways. As mentioned above, a suitable baffle may be placed so that the bath stream entering the chamber is deflected around the wall of the chamber, the chamber in this case being substantially circular in shape. Another method of imparting the required turbulent swirling motion is by using an air jet, which is preferably placed near the point where the bath, along with the filaments, enters the chamber and at a transverse angle to the bath conduit, preferably about 90°. The preferred method of imparting the turbulent swirling motion, however, is by means of a stream of bath which is jetted into the bath stream carrying the filaments. Preferably, the second bath stream is jetted into the first stream by means of an orifice located adjacent to the point of entrance of the first bath stream and positioned so that the second bath stream travels in a transverse direction to that of the first bath stream to deflect the filaments toward the side of the chamber.

In drawing the yarn away from the swirl-chamber, high tensions should be avoided to prevent the entanglements in the filaments from being partially or completely removed. The tensions normally encountered when using ordinary guides will cause no difficulty.

The swirl-chamber may be of any size and shape and may be varied depending on the processing conditions employed. The chamber is, however, preferably bowl-shaped and, for the processing of most textile yarns, is from 3 to 5 inches in diameter. The outlet for the bath and yarn may be rounded and is preferably centered in the bottom of the bowl, but this may be varied to some extent without harm, e.g., it may be located at one side of the chamber.

The random variations in the spacing, the length and the bulkiness of the bulky portions of the yarns of this invention result in fabrics having highly attractive surface effects. Such fabrics are highly desirable for use in such applications as wearing apparel and drapery materials.

Since many different embodiments of the invention may be made without departing from the spirit and scope thereof, it is to be understood that the invention is not limited by the specific illustrations except to the extent defined in the following claims.

I claim:

1. A blended bulky yarn comprising continuous wet-spun synthetic filaments intermingled with other continuous synthetic filaments, said yarn being looped and entangled at spaced intervals along the yarn length to form spaced bulky sections in the yarn, said bulky sections being separated from each other by an axial distance vary-

5

10

15

20

25

30

35

40

45

50

55

60

ing in completely random fashion and the bulkiness of said sections continuously varying in completely random fashion, the minimum variation in length being at least five-fold and the minimum variation in bulkiness being at least two-fold, the yarn in said sections separating said bulky sections comprising substantially straight filaments in compact even alignment.

2. The blended yarn of claim 1 wherein the wet-spun filaments comprise rayon and the other continuous filaments comprise polyethylene terephthalate.

3. A cross-dyed fabric of unusual appearance made from a yarn comprising continuous wet spun synthetic filaments intermingled with other continuous filaments of a different type looped and entangled at laterally aligned intermittent intervals along their length to form randomly spaced bulky sections along the yarn length, said bulky sections continuously varying in completely random fashion as to section length and bulkiness, the minimum variation in length being at least five-fold and the minimum variation in bulkiness being at least two-fold, the axial lengths between said bulky sections comprising substantially smooth, uncrimped closely aligned filaments, said bulky sections and lengths of aligned filaments co-operating to produce in said fabric a linen-like appearance with uneven roughened areas of varying size creating splash-like effects completely randomly scattered throughout said fabric corresponding to said bulky sections of said yarn.

4. The fabric of claim 3 in which the wet spun yarn filaments are of a rayon composition and the differing filaments are composed of polyethylene terephthalate.

5. A bulky yarn comprising continuous filaments each looped and entangled at laterally aligned intermittent intervals throughout the yarn length to form spaced bulky sections in the yarn, the spacing between said bulky sections varying in a random fashion, said bulky sections continuously varying in completely random fashion as to length and bulkiness, the minimum variation in length being at least five-fold, and the minimum variation in bulkiness being at least two-fold, the axial length between said bulky sections comprising continuous substantially unbukled filaments in a compact constant denier arrangement.

#### References Cited in the file of this patent

##### UNITED STATES PATENTS

|           |                  |                |
|-----------|------------------|----------------|
| 1,122,231 | Caldwell         | Dec. 22, 1914  |
| 1,165,819 | Ware             | Dec. 28, 1915  |
| 2,000,951 | Hodson           | May 14, 1935   |
| 2,255,246 | Fraser           | Sept. 9, 1941  |
| 2,451,504 | Mayo             | Oct. 19, 1948  |
| 2,700,866 | Strang           | Feb. 1, 1955   |
| 2,783,609 | Breen            | Mar. 5, 1957   |
| 2,854,814 | Burkholder       | Oct. 7, 1958   |
| 2,964,900 | Hicks            | Dec. 20, 1960  |
| 2,999,351 | Davenport et al. | Sept. 12, 1961 |
| 3,041,812 | Marshall         | July 3, 1962   |
| 3,042,482 | Woodell          | July 3, 1962   |
| 3,047,932 | Pittman et al.   | Aug. 7, 1962   |

##### FOREIGN PATENTS

|         |               |              |
|---------|---------------|--------------|
| 776,410 | Great Britain | June 5, 1957 |
|---------|---------------|--------------|